

# UNITED STATES PATENT OFFICE.

J. BRAINERD AND WM. H. BURRIDGE, OF CLEVELAND, OHIO.

## IMPROVEMENT IN TANNING.

Specification forming part of Letters Patent No. 25,315, dated September 6, 1859.

*To all whom it may concern:*

Be it known that we, JEHU BRAINERD and WILLIAM H. BURRIDGE, of Cleveland, in the county of Cuyahoga and State of Ohio, have invented new and useful Improvements in Tanning; and we do hereby declare that the following is a full and complete description of the same and of the ingredients employed therein.

The nature of our invention relates to the use of the herein-named mineral salts or their solution, whether the same be used in the manner set forth in a patent granted to us on the 7th day of June, 1859, or whether the said salts or their solutions be used in any stage of the process of tanning or mixed with solutions of tannin, as hereinafter set forth, either with or without the addition of aloes.

We prepare an infusion or decoction in a close vessel from hoarhound, (*Marrubium vulgare*), motherwort (*Leonurus cardiaca*) or other species of the *Labiatae*, or from catechu, (*Terra japonica*), or from the barks commonly used in tanning, or a mixture of these. To every gallon of the strong liquor thus prepared we add half a pound of common salt, ( $NaCl$ ), half a pound of alum, ( $Al_2O_3 \cdot 3SO_3 \cdot 24HO$ ), and one fluid ounce of chloride of zinc, ( $ZnCl \cdot Aq.$ ). It is not, however, important to preserve the exact proportions herein named, for either of these ingredients may be varied in its proportion to the others without materially changing the result. For tanning soft leather, from one-half to one ounce of pulverized aloes may be added.

The compound prepared as above constitutes our tanning-liquor.

Skins or hides that have been fitted for tanning in the ordinary way can be tanned by immersion in this compound in from six to forty days, according to the thickness of the skins or hides and strength of the liquor.

In carrying forward this process it will be found necessary to transfer the skins or hides to vats containing strong liquor, after that into which they have been first immersed has become exhausted, and to repeat this till they have become thoroughly tanned; or the liquor in the vats may be recruited in strength by adding new ingredients. It will generally be found advisable to give skins and hides their first immersion in a liquor that has been partially exhausted of its strength by previous immersion of skins or hides therein. It will also be found advantageous to frequently handle the skins and hides during their immersion in the vats.

What we claim as our improvement, and desire to secure by Letters Patent, is—

The use of the herein-described compound for tanning, consisting of a solution of the herein-named mineral salts in mixture with a solution of tannin, either with or without the addition of aloes.

J. BRAINERD.  
W. H. BURRIDGE.

Witnesses to J. Brainerd's signature:

EDM. F. BROWN,  
DANIEL BREED.

Witnesses to W. H. Burridge's signature:

C. H. MARTIN,  
F. G. MATHER.